

1

3,282,744

## CHROMATE CONVERSION COATING

Fred Corwin Goldsmith, Painesville, Ohio, assignor to  
The Lubrizol Corporation, Wickliffe, Ohio, a corpora-  
tion of Ohio  
No Drawing. Filed May 8, 1963, Ser. No. 278,990  
12 Claims. (Cl. 148—6.2)

The present invention relates to a composition adapted for the corrosion-proofing of metal articles. In a more particular sense, it relates to a convenient and economical method for inhibiting the corrosion of metal articles, especially ferrous metal articles and galvanized and/or phosphated ferrous metal articles.

It is known to treat metal articles, especially ferrous metal and galvanized ferrous metal articles, with aqueous phosphating solutions, aqueous chromic acid solutions, aqueous metal nitrite solutions, and the like to improve the corrosion resistance of the metal article and extend the useful life of a subsequently applied siccative top-coat such as a top-coat of paint, lacquer, enamel, varnish, synthetic resin, etc. One major shortcoming of known methods of corrosion-proofing has been noted, for example, in the automotive and household appliance industries, where ferrous metal, galvanized ferrous metal, or phosphated ferrous metal parts are invariably provided with a siccative top-coat of lacquer or enamel. It has been observed that when such a top-coat is scratched or scored during, for example, handling, forming, or assembling operations, the metal substrate becomes a focal point for corrosion and for a phenomenon known as "undercutting." Undercutting, or the loosening of the top-coat in areas adjacent to a scratch or score, causes a progressive flaking of the top-coat from the affected area. In severe cases, the undercutting may extend an inch or more from each side of the scratch or score, causing a loosening and subsequent flaking of the top-coat from a substantial portion, if not all, of the metal article.

Another shortcoming, particularly troublesome to the household washing machine industry, is the tendency of top-coated metal parts which come in contact with aqueous cleaning solutions such as aqueous solutions of common soap or synthetic detergent to develop blisters in the top-coat due to the corrosion of the metal substrate. Such blisters grow in size as the corrosion progresses and, in some instances, flake from the rest of the top-coat and thereby expose portions of the bare metal substrate.

It is an object, therefore, of the present invention to provide an improved corrosion-proofing composition for metal articles.

Another object is to provide a method for reducing the incidence of undercutting and blistering in top-coated metal articles.

Still another object is to provide metal articles which exhibit improved resistance to the ravages of corrosion.

These and other objects of the invention are realized by the provision of a composition adapted for the corrosion-proofing of metal articles which consists essentially of a dilute aqueous solution of

(A) partially reduced chromic acid in which the ratio of hexavalent chromium to trivalent chromium is within the range from about 0.5 to about 5, preferably from about 0.8 to about 3, and

(B) calcium dichromate;

in which solution from about 20 to about 80 percent and preferably from about 30 to about 70 percent of the chromium content thereof is contributed by component A, the remainder of the chromium content being contributed by component B.

Such dilute aqueous solution will generally contain

2

from about 0.01 to about 0.3 percent and more often from about 0.03 to about 0.1 percent of chromium present as components A and B.

In a preferred embodiment, the invention is directed to a composition adapted for the corrosion-proofing of metal articles which consists essentially of a dilute aqueous solution of

(A) partially reduced chromic acid prepared by reducing chromic acid with methanol, in which partially reduced chromic acid the ratio of hexavalent chromium to trivalent chromium is about 1, and  
(B) calcium dichromate;

which solution contains from about 0.03 to about 0.1 percent of chromium and in which solution about half of said chromium content is contributed by component A.

It has been found that components A and B act in a synergistic manner; that is, a combination of these components is much more effective in reducing corrosion than either component when used alone. When used to treat galvanized steel prior to the application thereto of a top-coat of paint or enamel, the corrosion-proofing composition of the present invention completely eliminates undercutting.

## COMPONENT A

As indicated previously, this component is partially reduced chromic acid in which the ratio of hexavalent chromium to trivalent chromium is within the range from about 0.5 to about 5, preferably from about 0.8 to about 3. It is known, as exemplified by U.S. Patents Nos. 2,768,104 and 3,063,877, to reduce chromic acid partially by means of oxidizable compounds such as formaldehyde, ethanol, glycol and other polyalcohols, phenol, hydroquinone, potassium iodide, etc., and then to use a dilute solution of such partially reduced chromic acid as a corrosion-proofing composition. The preparation of component A does not constitute the invention claimed herein and such preparation may be effected by known methods set forth in the cited patents or elsewhere in the literature. Example I of U.S. Patent 3,063,877, for example, describes the preparation of a partially reduced chromic acid (ratio of hexavalent chromium to trivalent chromium: 1.27) by the reaction below 180° F. of a solution of chromic acid (prepared by dissolving 170 pounds of CrO<sub>3</sub> in 40 gallons of water) with a solution of 48 pounds of 36.6 percent aqueous formaldehyde in 21 gallons of water. From the standpoint of convenience and economy, however, it is generally preferred to use methanol as the reducing agent for chromic acid in preparing component A. The following examples are presented to illustrate additional specific modes of preparing partially reduced chromic acid useful for the purposes of the present invention. These examples are presented for purposes of illustration only and are not to be construed as limiting the scope of the invention, except as the appended claims may require. Unless otherwise indicated, all parts and percentages are by weight.

## Example 1

60 432 parts of water is introduced into a reaction vessel and 550 parts of CrO<sub>3</sub> is added thereto over a period of 20 minutes at 27–32° C. The whole is heated to 93° C. over a period of 1.5 hours and a mixture of 29 parts of methanol with 29 parts of water is added thereto beneath the surface of the chromic acid solution over a period of 4 hours at 90–99° C. A very exothermic reaction occurs and the addition must be made carefully to avoid a too vigorous reaction. Approximately 40 parts of carbon dioxide is formed as a consequence of the complete oxidation of the methanol. After all of the methanol has been added, the whole is stirred for 1 hour at 96° C. The product, a concentrated aqueous solution of

partially reduced chromic acid, shows the following analyses.

|                                                    |       |
|----------------------------------------------------|-------|
| Percent chromium                                   | 28.45 |
| Percent hexavalent chromium                        | 19.55 |
| Percent trivalent chromium                         | 8.90  |
| Ratio of hexavalent chromium to trivalent chromium | 2.2   |

### Example 2

To 1100 grams of  $\text{CrO}_3$  dissolved in 2500 grams of water and heated to 90-100° C., there is added dropwise a mixture of 128 grams of methanol and 128 grams of water. The highly exothermic reaction maintains the temperature at 90-100° C. After all of the aqueous methanol has been added (approximately 8 to 10 hours required), the whole is stirred for an additional hour to insure complete reaction. The material in the reaction vessel is then diluted with sufficient water to yield 3 liters of solution. The resulting product, a concentrated aqueous solution of partially reduced chromic acid, shows the following analyses.

|                                                    |       |
|----------------------------------------------------|-------|
| Percent chromium                                   | 14.75 |
| Ratio of hexavalent chromium to trivalent chromium | 1.15  |

### Example 3

An experiment is carried out in the same manner set forth in Example 2, except that a mixture of 89.6 grams of methanol and 89.6 grams of water is employed. The resulting product, a concentrated aqueous solution of partially reduced chromic acid, shows the following analyses.

|                                                    |      |
|----------------------------------------------------|------|
| Percent chromium                                   | 14.9 |
| Ratio of hexavalent chromium to trivalent chromium | 1.68 |

### Example 4

An experiment is carried out in the same manner set forth in Example 2, except that a mixture of 48 grams of methanol and 48 grams of water is employed. The resulting product, a concentrated aqueous solution of partially reduced chromic acid, shows the following analyses.

|                                                    |       |
|----------------------------------------------------|-------|
| Percent chromium                                   | 15.45 |
| Ratio of hexavalent chromium to trivalent chromium | 3.0   |

## COMPONENT B

As indicated earlier, this component is calcium dichromate. Although anhydrous calcium dichromate ( $\text{CaCr}_2\text{O}_7$ ) may be employed as component B, it is generally more convenient to use a concentrated aqueous solution thereof, because such solution dissolves immediately in water upon mixing. For example, the reaction of a slurry of 1.72 parts of calcium hydroxide in 6.5 parts of water with 5.1 parts of  $\text{CrO}_3$  for about 8 hours at 110°-120° F. yields an aqueous concentrate containing 45 percent of calcium dichromate.

As noted hereinabove, the corrosion-proofing composition of this invention consists essentially of a dilute aqueous solution of components A and B. Such dilute solutions will ordinarily contain from about 0.01 to about 0.3 percent of chromium. When less than about 0.01 percent of chromium is present, the corrosion-proofing characteristics of the solution fall off quite rapidly. More than 0.3 percent of chromium can be present; however, the use of such larger content of chromium is uneconomical and, in most instances, is not attended by any substantial increase in the corrosion-proofing characteristics of the solution. Preferably, the chromium content of the solution will be within the range from about 0.03 to about 0.1 percent. Each of components A and B contributes to the chromium content of the solution. In order for the objects of the invention to be achieved, it

is important that from about 20 to about 80 percent and preferably from about 30 to about 70 percent of the chromium content of the solution be contributed by component A, with the remainder being contributed by component B. When components A and B are present in such amounts, they act in a synergistic manner to provide optimum corrosion-proofing characteristics. It is likewise important that the ratio of hexavalent chromium to trivalent chromium in component A be within the range from about 0.5 to about 5, preferably from about 0.8 to about 3.

A number of specific examples of aqueous corrosion-proofing compositions of this invention are given in Table I. They are prepared by simply dissolving the indicated components in water.

TABLE I.—DILUTE AQUEOUS CORROSION-PROOFING COMPOSITIONS OF THE INVENTION

| Example No. | Component A          |                                                                  | Component B (calcium dichromate), present in an amount to supply the indicated percent of chromium |
|-------------|----------------------|------------------------------------------------------------------|----------------------------------------------------------------------------------------------------|
|             | Identity             | Present in an amount to supply the indicated percent of chromium |                                                                                                    |
| 5           | Product of Example 2 | 0.025                                                            | 0.025                                                                                              |
| 6           | Product of Example 3 | 0.025                                                            | 0.025                                                                                              |
| 7           | Product of Example 4 | 0.025                                                            | 0.025                                                                                              |
| 8           | Product of Example 2 | 0.05                                                             | 0.025                                                                                              |
| 9           | Product of Example 3 | 0.075                                                            | 0.025                                                                                              |
| 10          | Product of Example 4 | 0.03                                                             | 0.09                                                                                               |
| 11          | Product of Example 2 | 0.09                                                             | 0.18                                                                                               |
| 12          | Product of Example 3 | 0.08                                                             | 0.08                                                                                               |

The treatment of the metal article with the corrosion-proofing composition of this invention may be accomplished in any one of several ways. The composition may be contacted with or applied to the article by spraying, brushing, dipping, flow-coating, roller-coating, etc., techniques, and the temperature of the composition may vary within wide limits, e.g., from room temperature or below to about 212° F. Higher temperatures such as 250° F., 300° F., or more may also be employed by the use of superatmospheric pressures. In general, best results are obtained when the temperature of the composition is within the range from about 60° F. to about 150° F. The time of contact between the metal article and the composition of this invention is not critical and may vary from as little as 5 or 10 seconds to as much as 10 minutes or more. In most instances a contact time between about 15 seconds to about 1 or 2 minutes suffices. For best results, the metal article should be thoroughly clean before it is contacted with the corrosion-proofing composition. Cleaning, if required, may be accomplished by known physical and/or chemical means which remove grease, dirt, oxides, and other surface contaminants.

After the metal article has been treated with the composition of this invention, it is dried. This can be done by allowing it to drain and dry at ambient temperature, by subjecting it to a current of hot air, by passing it through a heated zone, etc. The treated and dried metal article is then generally provided with a siccative top-coat such as a top-coat of paint, enamel, varnish, lacquer, synthetic resin, etc., to provide further protection and/or decorative effects. Such top-coat may be applied by conventional means such as spraying, brushing, dipping, roller-coating, etc., and then dried either by exposure to air or by means of a baking technique, depending on the nature of the siccative top-coat material.

The following experiments were carried out to determine the corrosion-proofing characteristics of compositions of this invention. They are presented for purposes of illustration only and are not intended to limit the scope of the invention, except as the appended claims may require. Unless otherwise specified, all parts and percentages are by weight.

5  
*Example 13*

Three clean, 4-inch by 12-inch panels of satin finish, galvanized 20-gauge SAE 1020 steel were spray-phosphated for one minute at 150° F. with an aqueous phosphating solution containing 0.091% of calcium ion, 0.029% of zinc ion, 0.71% of phosphate ion, 0.034% of nickel ion, and 0.13% of nitrate ion, and having a total acidity of 12.7 points (points total acidity represents the number of milliliters of 0.1 normal sodium hydroxide solution required to neutralize a 10 milliliter sample of the phosphating solution in the presence of phenolphthalein indicator). The phosphated panels were spray-rinsed with water for 15 seconds at room temperature and then spray rinsed for 15 seconds at room temperature, respectively, with a corrosion-proofing composition of this invention (Example 6; contains 0.05% of chromium) and two control solutions prepared by separately dissolving component A and component B of Example 6 in sufficient water to yield solutions containing 0.05% of chromium. For convenient identification, the panels were labeled, respectively, as panels E, F, and G. After the panels had been treated, they were dried in a current of hot (300° F.) air for 10 seconds and dipped in a gray, epoxy resin-based bake enamel. The top-coated panels were then baked in an oven for 10 minutes at 400° F. and subjected to the Tide Corrosion test. In this test, panels to be evaluated are immersed for 96 hours at 160° F. in an aqueous detergent solution consisting of water plus 1 percent of a synthetic detergent composition consisting of 53 parts of sodium pyrophosphate decahydrate, 19 parts of sodium sulfate, 20 parts of sodium alkylbenzene sulfonate, 7 parts of sodium metasilicate, and 1 part of sodium carbonate. Upon removal from the test solution, the panels are rated for blistering of the top-coat by means of ASTM Procedure D 714-56. The rating provides for the designation of the size of any blisters present on a scale of 0 to 10, wherein 0 represents large blisters and 10 represents no blisters. It also provides for the frequency of any blisters present as follows: dense=D, medium dense=MD, medium=M, and few=F.

The test results obtained on the several panels of this example are set forth in Table II.

TABLE II.—TIDE CORROSION TEST

| Top-Coated Panel          | Blister Size | Blister Frequency |
|---------------------------|--------------|-------------------|
| E (of the invention)..... | 10           | none              |
| F (control).....          | 8            | MD                |
| G (control).....          | 9            | F                 |

It will be noted that the panel which had been treated with a corrosion-proofing composition of this invention was superior to panels which had been treated with separate solutions of components A and B of said composition.

*Example 14*

Three clean, galvanized steel panels of the type described in Example 13 were spray-rinsed with water for 15 seconds at room temperature and then spray-rinsed for 15 seconds at room temperature, respectively, with a corrosion-proofing composition of this invention (Example 5; contains 0.05% of chromium) and two control solutions prepared by separately dissolving component A and component B of Example 5 in sufficient water to yield solutions containing 0.05% of chromium. For convenient identification, the panels were labeled, respectively, as panels H, I, and J. The panels were dried, top-coated, baked, and tested in the same manner set forth in Example 13.

The test results obtained on the several panels are shown in Table III.

## 6

TABLE III.—TIDE CORROSION TEST

| 5 | Top-Coated Panel | Blister Size | Blister Frequency         |                  |
|---|------------------|--------------|---------------------------|------------------|
|   |                  |              | H (of the invention)..... | I (control)..... |
|   | J (control)..... | 5            | 9                         | F                |
|   |                  |              | 8                         | MD               |
|   |                  |              | 5                         | MD               |

Again it will be noted that the panel which had been treated with a corrosion-proofing composition of this invention was superior to panels which had been treated with separate solutions of components A and B of said composition.

*Example 15*

Three clean, 4-inch by 12-inch panels of spangle finish, galvanized 20-gauge SAE 1020 steel were spray-rinsed with water for 15 seconds at room temperature and then spray-rinsed for 15 seconds at room temperature, respectively, with a corrosion-proofing composition of this invention (Example 5; contains 0.05% of chromium) and two control solutions prepared by separately dissolving component A and component B of Example 5 in sufficient water to yield solutions containing 0.05% of chromium. For convenient identification, the panels were labeled, respectively, as panels K, L, and M. The treated panels were dried in a current of hot (300° F.) air for 10 seconds and then sprayed with a white, alkyl resin-based bake enamel. The top-coated panels were baked in an oven for 20 minutes at 320° F., scribed with a sharp steel instrument to yield a vertical score extending one inch from the top of the panel to one inch from the bottom thereof, and subjected to the Salt Fog Corrosion test. The apparatus used for this test is described in ASTM Procedure B 117-57T. It consists of a chamber in which a mist or fog of 5 percent aqueous sodium chloride is maintained in contact with the test panels for a predetermined time (in the present case, 120 hours) at 95°±2° F. Upon removal from the test chamber, the top-coated panels are inspected and rated for undercutting. The "undercut rating" is the average loss of enamel from each side of the score expressed as a value which represents the number of thirty-seconds of an inch of such loss.

The results obtained in this test are shown in Table IV.

45 TABLE IV.—SALT FOG CORROSION TEST, 120 HOURS

| Top-coated panel:         | Undercut rating |
|---------------------------|-----------------|
| K (of the invention)..... | 0.0             |
| L (control).....          | 6.0             |
| M (control).....          | 7.0             |

It will be noted that the panel which had been treated with a corrosion-proofing composition of this invention showed no undercutting, whereas panels which had been treated with separate solutions of components A and B of said composition showed substantial loss of enamel due to undercutting.

*Example 16*

An experiment like that described in Example 15 was carried out, with the exception that the corrosion-proofing composition of the invention employed was that of Example 6 (contains 0.05% of chromium). The two control solutions were prepared by separately dissolving component A and component B of Example 6 in sufficient water to yield solutions containing 0.05% of chromium. For purposes of identification, the panels were labeled, respectively, as panels N, O, and P.

The test results are shown in Table V.

TABLE V.—SALT FOG CORROSION TEST, 120 HOURS

| Top-coated panel:         | Undercut rating |
|---------------------------|-----------------|
| N (of the invention)..... | 0.0             |
| O (control).....          | 9.0             |
| P (control).....          | 7.0             |

Again, the panel which had been treated in accordance with the present invention gave superior results.

## Example 17

An experiment like that described in Example 15 was carried out, with the exception that the corrosion-proofing composition of the invention employed was that of Example 7 (contains 0.05% of chromium). The two control solutions were prepared by separately dissolving component A and component B of Example 7 in sufficient water to yield solutions containing 0.05% of chromium. For purposes of identification, the panels were labeled, respectively, as panels Q, R, and S.

The test results are shown in Table VI.

TABLE VI.—SALT FOG CORROSION TEST, 120 HOURS

| Top-coated panel:    | Undercut rating |
|----------------------|-----------------|
| Q (of the invention) | 0.0             |
| R (control)          | 2.5             |
| S (control)          | 7.0             |

Superior results were again obtained with the panel which had been treated in accordance with the present invention.

## Example 18

Example 17 was repeated using plain steel panels instead of galvanized steel panels. The panel treated with the composition of this invention was labeled panel T; the control panels were U and V.

The test results are set forth in Table VII.

TABLE VII.—SALT FOG CORROSION TEST, 120 HOURS

| Top-coated panel:    | Undercut rating |
|----------------------|-----------------|
| T (of the invention) | 5.0             |
| U (control)          | 10.0            |
| V (control)          | 14.0            |

The experiment shows that the corrosion-proofing composition of this invention is effective in protecting plain steel as well as galvanized or phosphated steel.

In addition to their utility as corrosion-proofing compositions for application to the surfaces of ferrous metal articles, galvanized ferrous metal articles, and phosphated metal articles, the corrosion-proofing compositions of this invention are also useful in protecting non-ferrous metals and alloys thereof such as aluminum, magnesium, cadmium, copper, brass, bronze, white metal, etc., against corrosion. They are also useful in protecting plated metal surfaces such as copper-plated, nickel-plated, and cadmium-plated ferrous metal articles against corrosion.

What is claimed is:

1. A composition adapted for the corrosion-proofing of metal articles which consists essentially of a dilute aqueous solution of

(A) partially reduced chromic acid in which the ratio

of hexavalent chromium to trivalent chromium is within the range from about 0.5 to about 5, and  
 (B) calcium dichromate;  
 In which solution from about 20 to about 80 percent of the chromium content thereof is contributed by component A.

5 2. A composition in accordance with claim 1 which contains from about 0.01 to about 0.3 percent of chromium.

3. A composition in accordance with claim 1 wherein the ratio of hexavalent chromium to trivalent chromium in component A is within the range from about 0.8 to about 3.

4. A composition in accordance with claim 1 wherein from about 30 to about 70 percent of the chromium content thereof is contributed by component A.

5 5. A composition in accordance with claim 1 wherein component A is prepared by partially reducing chromic acid with methanol.

6. A composition adapted for the corrosion-proofing of metal articles which consists essentially of a dilute aqueous solution of

(A) partially reduced chromic acid prepared by reducing chromic acid with methanol, in which partially reduced chromic acid the ratio of hexavalent chromium to trivalent chromium is about 1, and

(B) calcium dichromate;  
 which solution contains from about 0.3 to about 0.1 percent of chromium and in which solution about half of said chromium content is contributed by component A.

7. A method of corrosion-proofing a metal article which comprises contacting said metal article with the composition of claim 1.

8. A method in accordance with claim 7 wherein the metal article is a ferrous metal article.

9. A method in accordance with claim 7 wherein the metal article is a galvanized ferrous metal article.

10. A method in accordance with claim 7 wherein the metal article is a phosphated metal article.

11. A metal article which has been corrosion-proofed in accordance with the method of claim 7.

12. A metal article in accordance with claim 11 which has been provided with a siccative top-coat.

45 References Cited by the Examiner  
 UNITED STATES PATENTS  
 2,773,623 12/1956 Schuster et al. ----- 148—6.2 X  
 2,868,679 1/1959 Pimbley ----- 148—6.2  
 3,053,702 9/1962 Schuster et al. ----- 148—6.2

ALFRED L. LEAVITT, Primary Examiner.

R. S. KENDALL, Assistant Examiner.

UNITED STATES PATENT OFFICE  
CERTIFICATE OF CORRECTION

Patent No. 3,282,744

November 1, 1966

Fred Corwin Goldsmith

It is hereby certified that error appears in the above numbered patent requiring correction and that the said Letters Patent should read as corrected below.

Column 7, line 3, for "comopsition" read -- composition  
--; column 8, line 28, for "0.3" read -- 0.03 --.

Signed and sealed this 5th day of September 1967.

(SEAL)

Attest:

ERNEST W. SWIDER

Attesting Officer

EDWARD J. BRENNER

Commissioner of Patents